

## UNITED STATES PATENT OFFICE

2,318,630

## LUBRICATING COMPOSITION

Carl F. Prutton, Cleveland, Ohio, assignor to The Lubri-Zol Corporation, Wickliffe, Ohio, a corporation of Ohio

No Drawing. Application August 8, 1938,  
Serial No. 223,694

5 Claims. (Cl. 252—45)

The present invention relates as indicated to lubrication and more particularly to methods of lubricating and lubricating compositions characterized by their ability to withstand extreme unit pressures between the bearing surfaces which the same are called upon to lubricate, without the disadvantages of instability and gum-forming tendencies which characterize many similar lubricating compositions now commonly available.

This application is a continuation in part of my copending applications Serial No. 737,070, filed July 26, 1934, and Serial No. 193,960, filed March 4, 1938.

It is a principal object of this invention to provide a lubricating composition utilizing certain compounds of sulphur as the means for providing the improved type of lubrication above identified, such compounds being used either in their pure state or admixed with lubricating compositions such as mineral oils and the like.

By "extreme pressures," as referred to above, is meant pressures of or in excess of 10,000 pounds per square inch, such pressures now being commonly encountered in hypoid gears, bearings, contact surfaces of cylinders and piston rings in internal combustion engines, and many other points. Such pressures tend to cause the rupture of the continuous "thick film" of lubricant which separates bearing surfaces under more moderate conditions. A region of "thin film" lubrication results which is also sometimes described as "boundary" lubrication.

It is therefore an object of my invention to provide a lubricating composition and method of lubricating which will afford efficient lubrication and protection to the relatively moving metallic surfaces under conditions of extreme pressure.

Other objects of this invention will appear as the description proceeds.

To the accomplishment of the foregoing and related ends, said invention, then, consists of the means hereinafter fully described and particularly pointed out in the claims, the following description setting forth in detail certain approved combinations of ingredients embodying my invention, such disclosed means constituting, however, but certain of various forms in which the principle of the invention may be used.

Briefly stated, my invention comprises the discovery that a certain class of sulphur compounds, namely the organic mono- and di-sulphides, although stable and relatively chemically inactive at ordinary temperatures and pressures, will, nevertheless, when present in a lubricant film and subjected to the conditions imposed on the bearing surfaces under abnormally high unit pressures, react with said surfaces to form a film which will prevent seizure and scoring at extreme pressures.

When used in conjunction with a mineral lu-

bricating oil it is obvious that generally only such amounts of the addition agent may be included as are soluble in the specified amount of oil. By the term "soluble" as herein used it is intended to indicate the ability to form not only true solutions but also any form of substantially permanently homogeneous composition when incorporated in mineral oil. With most of the compounds there is usually little difficulty, especially if the incorporation is effected in the manner described in Cornell Patent No. 2,042,880, and since relatively small proportions usually give improved results it is seldom of importance that the addition agents be oil-soluble in all proportions. Also, certain compounds are of value as gelling or bodying agents when used in amounts greater than are strictly soluble.

While for certain specialized uses the mono- and di-sulphides may be employed as the sole lubricant this invention contemplates that in general they will be employed as addition agents (either the sole addition agent or in combination with others) to mineral lubricating oils in amounts ranging from about .2% to about 20% by weight, based on the amount of mineral oil. From about 1/2% to 7%, or preferably from about 1% to about 5% will be found to be a desirable proportion for general use although larger amounts up to about 10% or more may be found more advantageous for certain uses. The proportion added, however, is often limited by the limit of solubility in the particular oil. The final products should contain an amount of the addition agent sufficient to increase the film strength of the lubricant, to a substantial degree. The required minimum amount will usually be found to be about 0.2%, in order that the lubricant may exhibit sufficient extreme pressure properties to be commercially feasible.

Although the oil base is referred to above as a mineral lubricating oil it is to be understood that any other suitable hydrocarbon lubricating oil, whether naturally occurring or synthetic may be employed as the oil base. For most purposes mineral lubricating oils having a viscosity from about 50 to 250 second Saybolt at 210° F. are entirely suitable, and for certain purposes, as for example gear lubrication, a viscosity range of 90 to 200 seconds is desirable.

It is also within the contemplation of this invention to provide the addition agent in the form of a concentrate in a suitable oil, said oil containing rather high percentages of the addition agent. Such concentrates are employed for future blending with a lubricating oil in the proportions desired for the particular conditions of use.

When still greater resistance to extreme pressure conditions is desired than that afforded by the addition agent of this invention alone, it may

often be found advantageous to employ a small amount of a separate organic halogen compound in the lubricant which will cooperate with the addition agent of this invention to increase the film strength (e. g. as indicated on the Almen Machine) to a degree greater than the sum of the effects of either addition agent when employed alone.

Since, in general, the loss of the addition agent by volatilization will be less for compounds having a low volatility, the vapor pressure of the compounds should, for most purposes, be less than atmospheric pressure at temperatures up to 140° C. It is usually desirable, especially for use in internal combustion engines, that the vapor pressure be less than atmospheric at temperatures up to 170° C. In the case of compounds which are stable at temperatures up to their boiling points, this condition may be expressed by stating that the boiling point of the compound should, in general, be higher than 140° C., and for certain uses, such as in internal combustion engines, higher than 170° C.

Examples of the types of compounds which may be employed in accordance with my invention are the di-aryl and di-alkyl sulphides and di-sulphides and also sulphides and di-sulphides containing both an alkyl and an aryl radicle, e. g.:

Di-alkyl sulphides, e. g.:

Di-amyl sulphide

Di-lauryl sulphide

Arylated alkyl sulphides, e. g.:

Dibenzyl sulphide

Di-aryl sulphides, e. g.:

Di-phenyl sulphide

Di-alkyl disulphides, e. g.:

Di-ethyl disulphide

Di-n-butyl disulphide

Di-amyl disulphide

Arylated alkyl disulphides, e. g.:

Di-benzyl disulphide

Di-phenyl di-ethyl disulphide

(C<sub>6</sub>H<sub>5</sub>—C<sub>2</sub>H<sub>4</sub>—S)<sub>2</sub>

Di-methyl di-benzyl disulphide

(CH<sub>3</sub>—C<sub>6</sub>H<sub>4</sub>—CH<sub>2</sub>—S)<sub>2</sub>

Di-aryl disulphides, e. g.:

Di-phenyl disulphide

Alkylated aryl disulphides, e. g.:

Di-tolyl disulphide

Di-xylyl disulphide

Mixed aryl-alkyl sulphides and disulphides

methyl phenyl sulphide and disulphide

ethyl phenyl sulphide and disulphide

amyl phenyl sulphide and disulphide

Certain classes of these sulphur compounds may be defined as:

(1) Disulphides having the general formula:

R—S—S—R<sub>1</sub>, wherein R and R<sub>1</sub> represent substituents selected from the group consisting of alkyl groups or hydrocarbon phenyl groups.

(2) Organic sulphides having the general formula R—S—R<sub>1</sub>, wherein R and R<sub>1</sub> represent (a) alkyl groups containing at least 5 carbon atoms each, or (b) phenyl groups or alkyl groups containing from 5 to 6 carbon atoms each.

The alkyl derivatives of the aryl disulphides (e. g., di-xylyl disulphide) and the aryl derivatives of alkyl disulphides (e. g., diphenyl diethyl disulphide) are particularly desirable not only because of their effectiveness but also because of their ready solubility in mineral oils.

Obviously the addition agent chosen should be sufficiently oil-soluble so that the amount used will remain in solution under the operating conditions encountered, preferably, for automotive and other ordinary applications, at temperatures down to 20° below zero. The oil solubility will depend to some extent upon the character of the oil, usually being higher for the less viscous Gulf Coastal oils and lower for the viscous Pennsylvania oils in the case of mineral oils.

From the point of view of solubility, the most advantageous conditions would generally result from the use of a compound which is liquid and miscible with the oil base used. An example of such compound is diphenyl sulphide.

While mineral oil generally is the principal ingredient of the lubricant, it is not essential that it be the only ingredient other than the addition agent, provided that there be no additional ingredient which is incompatible with such addition agent. It is within the contemplation of this invention to include, if necessary or desirable, such other addition agents as are commonly added to improve the viscosity index or cold test of the lubricant and a lubricating composition according to this invention which also has a separate oiliness increasing agent has been found to be especially effective.

While the lubricating compositions which have been described herein as illustrating one embodiment of the invention have been generally referred to as "oils," i. e., liquids, this invention is, however, also especially applicable to the solid and semi-solid types of lubricants commonly referred to in the trade as greases, bodied oils, etc., and which may contain soaps such as sodium, calcium, lead and aluminum naphthenates, stearates and oleates.

It should be noted that the addition agents of this invention are relatively chemically stable and will therefore have no corrosive action upon the metal surfaces with which the lubricant comes in contact.

Other modes of applying the principle of my invention may be employed instead of the one explained, change being made as regards the composition and method herein disclosed, provided the ingredients or steps stated by any of the following claims or the equivalent of such stated ingredients or steps be employed.

I therefore particularly point out and distinctly claim as my invention:

1. An improved lubricating composition comprising a major proportion of mineral lubricating oil the film strength of which is increased by the inclusion therein of a liquid, oil-miscible organic sulphur compound selected from the class consisting of the organic sulphides and organic di-sulphides.

2. An improved lubricating composition comprising a major proportion of mineral lubricating oil the film strength of which is increased by the inclusion therein of a liquid, oil-miscible organic sulphur compound selected from the class consisting of the aryl sulphides and aryl di-sulphides.

3. An improved lubricating composition comprising a major proportion of mineral lubricating oil the film strength of which is increased by the inclusion therein of a liquid, oil-miscible organic sulphur compound selected from the class consisting of the aryl sulphides.

4. An improved lubricating composition comprising a major proportion of mineral lubricating oil, the film strength of which has been in-

creased by the inclusion therein of a minor amount of a liquid, oil-miscible organic sulphur compound selected from the class consisting of organic sulphides and disulphides.

5. An improved lubricating composition comprising a major proportion of mineral lubricating oil, the film strength of which has been in-

creased by the inclusion therein of a minor amount of a liquid, oil-miscible organic sulphur compound selected from the class consisting of organic sulphides and disulphides of the type in which the sulphur is attached to a benzenoid ring structure.

CARL F. PRUTTON.